

## UNITED STATES PATENT OFFICE.

GEORGE D. CHAMBERLAIN, OF ASHLAND, KENTUCKY, ASSIGNOR TO R. T. VANDERBILT COMPANY, INCORPORATED, OF NEW YORK, N. Y., A CORPORATION OF NEW YORK.

## PICKLING OF METALS.

No Drawing.

Application filed February 19, 1927. Serial No. 189,873.

This invention relates to the pickling and cleaning of metals, and particularly to the pickling of iron or steel, to remove scale therefrom, although the invention is of more 5 or less general application to the cleaning or pickling of metals such as iron or steel for the removal of oxides or scale therefrom.

The pickling or cleaning of iron or steel is commonly effected by means of acid pickling 10 or cleaning baths which remove the scale or oxide from the metal. The pickling baths commonly employed are acid baths which often attack the metal as well as the scale. This action on the metal is undesirable and 15 objectionable, involving not only excessive consumption of acids, but also corrosion or dissolving of metal and tending to give a rough or pitted surface.

The present invention provides an improved bath for pickling and cleaning metals 20 and also an improved process of pickling or cleaning the metal in which the acid pickling bath has incorporated therein a small amount of an inhibiting amine.

25 I have found that the addition of a small amount of certain amines prevents or retards or inhibits the attack of the acid pickling bath on the metal without interfering with the removal of scale or oxide by the acid bath.

30 The agents which are added to the cleaning or pickling bath, according to the present invention, include various of the amines which produce this inhibiting effect. Among these may be mentioned dibenzylaniline



dibenzylamine  $(\text{C}_6\text{H}_5\text{CH}_2)_2\text{NH}$ , 1,8-naphthylene diamine 1:8  $\text{CH}_{10}\text{H}_6(\text{NH}_2)_2$ , and triphenylguanidine  $(\text{C}_6\text{H}_5\text{NH})_2\text{C}:\text{N}(\text{C}_6\text{H}_5)_2$ .

40 I have found that these amines produce the desired inhibiting effect when used alone in the acid bath, and have also found that this inhibiting effect may also be produced by certain amines together with other compounds such as dibenzylaniline and thiocarbanilid.

The acid pickling baths with which the agents mentioned are used may be acid baths such as are commonly employed for pickling 50 or cleaning iron and steel, containing for example about ten percent of sulfuric acid. Such baths are gradually impoverished by the action of the acid in removing the scale or rust and their content of ferrous sulfate 55 increases until the bath becomes too weak or

too concentrated in ferrous sulfate for further use. Instead of using sulfuric acid baths, other acid baths can be used, including acid sulfate baths.

The amount of the inhibiting amine added 60 to the bath for carrying out the pickling or cleaning operation can be varied. In general, only a small amount of such a compound is required, for example, a small fraction of one percent. In the case of dibenzylaniline, for 65 example, about two to five pounds of the compound can be employed for each ton of sixty degree Baumé acid used in the pickling bath. A pickling bath including the same percentage of any of the other inhibiting amines 70 mentioned above likewise gives satisfactory results.

The carrying out of the pickling or cleaning operation may be the same as in ordinary 75 practice. For example, the pickling can be carried out continuously by passing the material to be pickled, such as wire or sheets, through a number of baths in a regulated manner; or by immersing the article to be pickled in the pickling bath for a suitable period of 80 time. The temperature of the bath can be varied, ordinarily being around 150 to 180° F. The pickling bath may be replenished by the addition of further amounts of acid until the iron sulfate reaches too great a concentration. 85

The addition of the inhibiting amine to the bath prevents or retards or inhibits the action of the acid bath on the metal without interfering with the removal of scale or oxide. The formation of hydrogen by the action of the 90 acid bath on the metal is also reduced and the production of acid mist or fumes also greatly reduced. There is also a saving in the acid as well as a protection of the metal. The reduced amount of action of the acid on the 95 metal and the reduction in amount of hydrogen produced correspondingly reduces the amount of hydrogen absorbed by the metal.

The employment of the inhibiting amine in the pickling or cleaning operation, according 100 to the present invention, involves but small additional expense and results in advantages in operation, economy of acid, protection of the metal from attack, etc., which materially improve the pickling and cleaning operation.

In the claims the word "amine" is used in a strict sense and refers to nitrogenous compounds in which the nitrogen is linked to hydrocarbon radicals, e. g. alkyl, aryl, aralkyl, etc. as distinguished from amides in 110

which one bond of the nitrogen is satisfied by an acid group, such as the C:O group in acetamide or the C:S in thiourea.

I claim:—

5. 1. The method of cleaning or pickling metals which comprises subjecting the same to a non-oxidizing mineral acid pickling or cleaning bath and inhibiting the chemical action of the acid on the metal without interfering with the removal of scale or oxide, and thereby reducing the formation of hydrogen and the production of acid mist and effecting an economy in the acid consumed, by incorporating in the acid bath a small amount of an inhibiting amine.

10. 2. The method of pickling or cleaning iron or steel which comprises subjecting the same to an acid pickling bath containing sulfuric acid and inhibiting the chemical action of the acid on the metal without interfering with the removal of scale or oxide, and thereby reducing the formation of hydrogen and the production of acid mist and effecting an economy in the acid consumed, by incorporating in the acid bath a small fraction of one per cent of an inhibiting amine.

15. 3. The method of cleaning or pickling metals which comprises subjecting the same to a non-oxidizing mineral acid pickling or cleaning bath and inhibiting the chemical action of the acid on the metal without interfering with the removal of scale or oxide, and thereby reducing the formation of hydrogen and the production of acid mist and effecting an economy in the acid consumed, by incorporating in the acid bath a small amount of dibenzylaniline.

20. 4. The method of pickling or cleaning iron or steel which comprises subjecting the same to an acid pickling bath containing sulfuric acid and inhibiting the chemical action of the acid on the metal without interfering with the removal of scale or oxide, and thereby reducing the formation of hydrogen and the production of acid mist and effecting an economy in the acid consumed, by incorporating in the acid bath a small fraction of one per cent of dibenzylaniline.

25. 5. The method of cleaning or pickling metals which comprises subjecting the same to a non-oxidizing mineral acid pickling or cleaning bath and inhibiting the chemical action of the acid on the metal without interfering with the removal of scale or oxide, and thereby reducing the formation of hydrogen and the production of acid mist and effecting an economy in the acid consumed, by incorporating in the acid bath a small amount of an inhibiting amine containing the group —NR<sub>2</sub> in which R is an aralkyl radical.

30. 6. The method of cleaning or pickling metals which comprises subjecting the same to a non-oxidizing mineral acid pickling or cleaning bath and inhibiting the chemical action of the acid on the metal without interfering

with the removal of scale or oxide, and thereby reducing the formation of hydrogen and the production of acid mist and effecting an economy in the acid consumed, by incorporating in the acid bath a small amount of an inhibiting amine of the formula R<sub>2</sub>NR' where R is an aralkyl radical and R' is an aromatic radical or hydrogen.

7. The method of cleaning or pickling metals which comprises subjecting the same to a non-oxidizing mineral acid pickling or cleaning bath and inhibiting the chemical action of the acid on the metal without interfering with the removal of scale or oxide, and thereby reducing the formation of hydrogen and the production of acid mist and effecting an economy in the acid consumed, by incorporating in the acid bath a small amount of an inhibiting amine of the formula R<sub>2</sub>NR' where R is an aralkyl radical and R' is an aryl radical.

8. The method of cleaning or pickling metals which comprises subjecting the same to a non-oxidizing mineral acid pickling or cleaning bath and inhibiting the chemical action of the acid on the metal without interfering with the removal of scale or oxide, and thereby reducing the formation of hydrogen and the production of acid mist and effecting an economy in the acid consumed, by incorporating in the acid bath a small amount of a dibenzylated amine.

9. The method of pickling or cleaning iron or steel which comprises subjecting the same to an acid pickling bath containing sulfuric acid and inhibiting the chemical action of the acid on the metal without interfering with the removal of scale or oxide, and thereby reducing the formation of hydrogen and the production of acid mist and effecting an economy in the acid consumed, by incorporating in the acid bath a small fraction of one per cent of dibenzylamine.

10. The method of cleaning or pickling metals which comprises subjecting the same to a non-oxidizing mineral acid pickling or cleaning bath and inhibiting the chemical action of the acid on the metal without interfering with the removal of scale or oxide, and thereby reducing the formation of hydrogen and the production of acid mist and effecting an economy in the acid consumed, by incorporating in the acid bath a small amount of dibenzylaniline together with thiocarbanilid.

11. The method of pickling or cleaning iron or steel which comprises subjecting the same to an acid pickling bath containing sulfuric acid and inhibiting the chemical action of the acid on the metal without interfering with the removal of scale or oxide, and thereby reducing the formation of hydrogen and the production of acid mist and effecting an economy in the acid consumed, by incorporating in the acid bath a small fraction of one

per cent of dibenzylaniline together with thiocarbanilid.

12. A non-oxidizing mineral acid bath for pickling or cleaning metals containing a small amount of an inhibiting amine. 5

13. A bath for pickling or cleaning metals containing sulphuric acid and a small fraction of one per cent of an inhibiting amine.

14. A non-oxidizing mineral acid bath for pickling or cleaning metals containing a small amount of a dibenzylated amine. 10

15. A non-oxidizing mineral acid bath for

pickling or cleaning metals containing a small amount of an amine containing the group —NR<sub>2</sub> in which R is an aralkyl radical. 15

16. A non-oxidizing mineral acid bath for pickling or cleaning metals containing a small amount of an inhibiting amine of the formula R<sub>2</sub>NR' where R is an aralkyl radical 20 and R' is an aryl radical.

In testimony whereof I affix my signature.

GEORGE D. CHAMBERLAIN.